

## UNITED STATES PATENT OFFICE.

THOMAS HAROLD FAIRBROTHER AND ARNOLD RENSHAW, OF MANCHESTER, ENGLAND, ASSIGNORS TO BRITISH DYESTUFFS CORPORATION LIMITED, OF MANCHESTER, ENGLAND, A CORPORATION OF GREAT BRITAIN AND IRELAND.

## MILDEW PROOFING OF FIBROUS MATERIAL.

No Drawing. Application filed December 17, 1926, Serial No. 155,545, and in Great Britain July 24, 1925.

Cotton materials when manufactured and finished in the usual way are liable to damage by mildew, especially when transported or stored in damp, warm climates, and the same is true with reference to other textile goods such as artificial silk and to materials such as paper, leather, leather-cloth, and the like. We have found that this fault can be overcome by suitably applying in the process of manufacture or finishing a solution of an alkaline salt of a highly halogenated phenol as hereinafter more particularly defined.

Alkali salts of mono- and di-halogenated phenols have previously been proposed for use as disinfectants and antiseptics. We have found that alkali salts of tri- and higher halogenated derivatives of phenol, cresols and naphthols have a destructive action upon the organisms of mildew which amounts to specificity when compared with the feeble action of the mono- and di-halogen derivatives. Alkaline salts, such as the sodium salt of 2:4:6:trichlorophenol, are particularly useful. Thus we have found that a solution of sodium phenate in a dilution of 1 in a 1000 does not restrain mildew growth, whilst para-chlor-sodium-phenate restrains growth under the same conditions in a dilution of 1 to 5000, and the highly halogenated tri-chlor-sodium-phenate shows a restraining action even when the dilution is as great as 1 in 40,000, and in a dilution of 1 in 5,000, the spores of the fungus which causes mildew are killed. Tri-brom-sodium-phenate shows a similar restraining action, as do also the halogenated cresols containing more than two atoms of halogen in the molecule. The free tri-halogenated phenols have been proposed as disinfectants and as medicinal preparations but the specific action of alkali salts of these tri-halogenated phenols on mildew organisms is new.

We apply these observations in the manufacture of cotton and other materials, particularly such as are liable to be exposed to moisture and a hot climate, and thus obtain a product which is immune from the attacks of mildew to a very high degree. For this purpose the yarn or other material is finished by immersion in a bath containing in solution the sodium salt of the halogenated phenol containing more than two atoms of

halogen in the molecule, in a concentration between, say, 1 in 100 1 in 1000, or by spraying the material with this solution. If the material is to be dyed, the halogenated phenol compound may be added to the dyebath to give a solution of similar concentration when it is taken up by the material to some extent along with the dye. This is particularly useful in the case of woolen cloths.

In the manufacture of paper, the halogenated phenol can be added to the pulp before filtration. In this way, papers are obtained which are particularly valuable for use:—

- (a) As wall-paper.
- (b) Paper used in connection with storage, and transportation of foodstuffs.
- (c) Paper used in legal documents.
- (d) Paper tubes.

The halogenated phenol can also be added to the size used for paper and other materials.

In the manufacture of artificial silk such as viscose silk or other cellulose product, the halogenated phenol is preferably added to the solution from which the cellulose is precipitated, when it remains to a great extent in the fibre obtained, and renders the fibre resistant to mildew.

What we claim and desire to secure by Letters Patent is:—

1. The improvement in the mildew-proofing of organic fibrous materials which consists in applying to the said materials a solution of an alkaline salt of a halogenated phenol containing more than two atoms of halogen to the molecule whereby they are protected from damage by mildew.

2. The improvement in the mildew-proofing of organic fibrous materials which consists in applying to the said materials during the manufacture thereof a solution of an alkaline salt of a halogenated phenol containing more than two atoms of halogen to the molecule whereby they are protected from damage by mildew.

3. The improvement in the mildew-proofing of organic fibrous materials which consists in applying to the said materials a solution of an alkaline salt of trichlorophenol whereby they are protected from damage by mildew.

4. The improvement in the mildew-proof-

ing of organic fibrous materials which consists in applying to the said materials a solution of an alkaline salt of 2:4:6:trichlorophenol whereby they are protected from damage by mildew.

5. The improvement in the mildew-proofing of organic fibrous materials which consists in applying to the said materials a solution of the sodium salt of 2:4:6-trichloro-

phenol whereby they are protected from 10 damage by mildew.

6. Mildew proof organic fibrous materials containing an alkaline salt of a trichlorophenol.

In testimony whereof we affix our signatures.

THOMAS HAROLD FAIRBROTHER.  
ARNOLD RENSHAW, M. D.